

Sept. 22, 1936.

A. GUTZWILLER

2,055,459

PROCESS FOR MAKING ASPHALT

Filed Aug. 1, 1932



Inventor:

Adolf Gutzwiller

By his Attorney:

John G. Gutzwiller

## UNITED STATES PATENT OFFICE

2,055,459

## PROCESS FOR MAKING ASPHALT

Adolf Gutzwiller, Amsterdam, Netherland, assignor to Shell Development Company, San Francisco, Calif., a corporation of Delaware

Application August 1, 1932, Serial No. 627,206  
In the Netherlands August 4, 1931

## 11 Claims. (Cl. 196—74)

This invention relates to the art of making blown asphalts and is more particularly concerned with a continuous method of producing asphaltic materials allowing flexible control of the treatment.

It is well known in the art that the properties of manufactured asphalts can be regulated by the conditions of the oxidizing treatment to which the raw materials are subjected during the manufacturing processes. A number of treating methods and apparatus are known at present, whereby various carbonaceous residues are subjected to oxidation and evaporation, or distillation, for producing asphalts of the desired qualities. Among the properties most commonly determining the quality of an asphaltic product, or its suitability for any particular use, can be mentioned: softening point, viscosity, flash point, penetration-temperature relation and ductility-temperature relation. Each of the well known uses of asphaltic materials, such as paving, roofing, pipe-coating, etc., requires a more or less definite set of properties which must be possessed by the material most suitable for the particular service in question. In order to obtain a product possessing a predetermined set of characteristics, it is necessary to maintain in each individual case of operation a definite combination of certain operating conditions, such as temperatures to which the material is subjected during treatment and the rate and the extent of oxidation. Other conditions being equal, the reaction of oxidation and its extent are markedly influenced by the composition of the material being treated, by its temperature at the time of oxidation, by the mass ratio of the oxidizing agent and the material treated at the oxidation zone, and by the time allowed for the oxidation to take place. The total effect of these factors upon the properties of the product is so pronounced, that the accurate control of the process is one of the most important requirements of an asphalt blowing plant.

It is an object of this invention to provide a process for manufacturing blown asphalt which can be easily adapted to the requirements of various feeds or different specifications of the finished product.

It is another object of this invention to provide a continuous process whereby a blown asphalt can be produced and its properties accurately adjusted to meet a set of fixed requirements.

The essential features of the new process will readily be understood from the following description illustrated by the attached drawing.

55 In carrying out this invention in practice, a

petroleum residue, produced by distillation, or cracking, or chemical treatment, or a coal tar, or any other suitable carbonaceous material can be used as charging stock. The material is continuously charged from a source not shown to a 5 heating coil 1, wherein the temperature of the material is raised to a suitable point, not exceeding cracking temperature, and preferably within the limits of 460-550° F. The raw material may be preheated before it reaches heater 1 by heat 10 exchange with hot media, such as the products leaving stills 4 and 12. The heated material is conducted through a pipe 2 to a perforated coil 3 positioned near the bottom of a blowing still 4; I found it advantageous to have coil 3 perforated 15 at the bottom, instead of at the top, as sediment carried by the liquid material is readily removed from the coil through the perforations, no sediment is allowed to settle and plug the perforations from outside, and greater stirring effect in still 4 20 is produced. On its way through the line 2, the hot material is mixed with air introduced under a suitable pressure through a pipe 5; although other chemically active gases or vapors can be used at this point, air is most commonly employed, and for the purpose of illustration, its 25 use is described in this specification.

A thorough mixing of air and liquid material takes place in pipe 2 and coil 3; the mixing occurring in the pipe 2 can be intensified, if desired, 30 by introducing the air into the oil stream in said pipe through a spraying nozzle. The mixture of the hot material and the air is discharged in a finely divided state from the coil 3 into still 4, wherein a suitable level of liquid is maintained 35 by means of overflow pipes 5', having a common header 6. At the temperature of the still 4, the light components of the treated material together with unconsumed gases separate from the liquid and are removed through pipe 7 to condenser 8 40 and to storage, not shown. The remaining air-blown residue is continually withdrawn, preferably near the surface of the pool in the still 4, and forced by a pump 9 through a heating coil 10, positioned either in a separate heater, or in 45 the heater containing coil 1.

It may be desirable in some cases to withdraw the air-blown product through an overflow pipe 5" or pipe connection 27 while maintaining the liquid level as indicated on the drawing or the 50 level may be lowered. Also the air-blown material from still 4 may be removed directly to storage through pipe 22 and heat exchanger 23, water or other fluid, such as incoming feed, being used to extract heat in the heat exchanger; 55

or it may be drained through either line 27 or 28. The liquid material withdrawn from still 4 usually contains a certain amount of dispersed gas, and I found it of considerable advantage to have this entrained gas separated from the air-blown material before passing the gas-free liquid to the pump 9 and heating coil 10. A gas separator 30 is used to separate the gas from the liquid; this gas separator 30 is positioned between the header 10 6 and pump 9 and is provided with a gas vent 31 and liquid trap 32. The liquid trap, or separator, can be of any well known and suitable construction. A by-pass 33 serves to convey the air-blown material, when the separation of gas 15 from the liquid is not deemed desirable, such as in the case of running this material directly to storage.

From the coil 10 the air-blown asphalt is passed on through line 11 and discharged into an evaporator 12 provided with rectifying means 13. Steam is injected into the evaporator 12 through a coil 15, preferably below the liquid level 14, which level is maintained at the desired height by liquid level controller 16. In the evaporator 25 12 a thorough contact is obtained between steam and the material being treated, and further separation of the more volatile components from the treated material is effected. The vapors are conducted out of the evaporator through pipe 17, condenser 18, and water separator 19, and the 30 substantially water-free condensate is pumped to storage not shown. The rectified steamed material is continually removed from the bottom of the evaporator 12 through a pipe 20, cooled in a heat exchanger 21, water or other fluid, such as incoming feed, being used to cool the material in the heat exchanger, and run to storage. A portion of the rectified asphalt may be recirculated through the evaporator 12 by means of a 35 pump 34 and a pipe connection 35, or it may be returned to the heating coil 1 by means of a pipe connection 36. Coil 10 may be wholly or partially by-passed through line 26.

As a modification of the steam treatment of air-blown asphalt, I have sometimes found it desirable to inject steam into coil 10 through a pipe 37. This mixing of steam with the air-blown material just before passing it through a heating zone has a decided carbonization-inhibiting effect.

A system of valves is provided throughout the apparatus described to properly control the flow of liquids and vapors.

Difficulties frequently encountered in the manufacture of blown asphaltic materials reside in the control of the temperature of oxidation to which the material undergoing treatment is subjected, and it is one of the objects of this invention to improve the method of this control.

One of the features of this process is the preferred method of introducing the air into the system after the heating coil but before the still. It has been known in the art to inject air directly into the still, or into the heating coil, or into the incoming charge before it enters the heating coil. Either of these methods has been practiced for some time with varying degree of success. Certain unavoidable difficulties have been found, however, to accompany these methods. The injection of air before or into the heating coil tends to cause undesirable carbonization of the material undergoing treatment, due, perhaps, to relatively high concentration of air at the points of high skin temperatures along the walls 75 of the heating coil. The pressures required for

injecting air before or into the heating coil are usually much higher than those employed in the present method.

Referring now to the method of injecting the air directly into the still, difficulties of other character have been encountered. When a relatively large body of oxidized or partly oxidized material is maintained in the still, the incoming charge becomes immediately diluted upon entering the still. It has been found that under these conditions a materially greater amount of air was required to effect the same degree and rate of oxidation, as obtained by a thorough mixing of the air with the hot raw liquid material just before the mixture is sprayed in the still. A greater quantity of undesirable distillate was produced when using the former method, and the uniformity of the air-blown residual material was difficult to maintain. My preferred method avoids the difficulties of both systems.

As has been described hereinbefore, the reacting mixture is, in this process, introduced into the still 4. To control the reactions taking place in this still, provisions are made:

- (1) to regulate the temperature of the heated material leaving the heating coil 1,
- (2) to regulate the gas flow in line 5,
- (3) to regulate the time of contact between the oxidizing gas and liquid asphalt, and
- (4) to regulate the composition of the material being treated.

While provisions (1) and (2) may be carried out in any conventional manner, it is the purpose of this invention to control the time of contact between the oxidizing gas and the liquid material by maintaining a suitable level of liquid in the still 4. Preferably, this still 4 is a vertical cylindrically shaped chamber provided with means for continuously introducing the reacting substances and withdrawing the resulting products. The use of such a still has been found much more advantageous than the use of the conventional horizontal chambers on account of the greater range available for varying the depth of liquid in such vertical still. Almost any desired degree of exhaustion of the active gas can be obtained by varying the liquid level, thus materially reducing the gas consumption.

It should be noted in this connection, that the vapor space in the still 4, contains, besides more volatile components of the asphaltic material, the residual gas substantially comprising only the inert portion of the gas injected through 5; it is readily seen, therefore, that the conditions prevailing in the still 4 are such that the lighter components of the asphaltic material are exposed only to the action of substantially non-oxidizing atmosphere, thus minimizing the carbonization of the material in the still 4.

It should be noted, furthermore, that the perforated coil 3 is continually and completely submerged in the liquid material; this eliminates conditions favorable for the formation of a highly viscous, sometimes solid, deposit of heavy material on said coil, which normally occurs when the coil is positioned at the top of the still and surrounded by air.

Due to the exothermic character of the oxidation reactions taking place in the still 4, the temperature of the liquid material is further raised, after being heated in coil 1. It has been found, that in order to avoid excessive carbonization of the treated material the temperature in the still 4 should preferably not exceed 550° F. In order to control this phase of the process, a portion of the

air-blown material may be continually recirculated by means of pipe connection 25, so that the raw material is somewhat diluted before being subjected to oxidation, and the heat of reaction per unit of reacting mass is thereby suitably regulated.

In certain cases it may be advisable to carry out the oxidation reaction at a somewhat diminished rate. Although it may be possible to realize this by regulating the rates of liquid and air flows through coil 1 and pipe 5, as well as by recirculation of the air-blown asphalt through line 25, and/or by a proper adjustment of the liquid level in still 4, it is preferred to provide an additional means for this purpose; viz. recirculation of a portion of the air-blown material from the still 4 to the coil 1 by means of a pipe 29. The raw material is diluted in this case prior to being heated, and the temperature and thereby the rate 20 of oxidation in the still 4 is accordingly reduced.

While the different properties of the air-blown material can be varied within rather wide limits by the process steps described hereinbefore, often it is found difficult to obtain the desired product 25 and to maintain the normal rate of production at the same time. It has been found, that, by incorporating in this process a step wherein the air-blown asphalt is further heated and steam treated the range of variation of the properties of the 30 finished asphalt is considerably expanded, the quality of the product improved, and a greater throughput realized. As has been described, the heating coil 10 is used to raise the temperature of the air-blown asphalt; the temperature of the 35 heated material after coil 10 preferably should not exceed 600° F., which in the absence of the chemically active gas at this stage of the treatment is a safe limit, below which extensive coking does not occur. The advantages of having the 40 steam still directly connected to the blowing still reside in the manner in which the composition of the feed in pipe 11 is controlled; this control is carried out by means of pipe connections 26 and 24, whereby oxidized, or unoxidized, material may 45 readily be introduced into line 11 to properly adjust the characteristics of the steam-rectified asphalt. Further continuous recirculation of a portion of the steamed asphalt through the steam still by means of line 35 has a marked effect upon 50 the ease with which various combinations of melting point, penetration and ductility of the finished product can be obtained.

It should be noted that although the use of coil 10 is specifically mentioned in the above description of my process and apparatus, I have found that, when no serious heat losses take place between stills 4 and 12, during treatment of certain types of oils, it is possible to dispense with the heating coil 10 and/or the gas-separator 30, and 60 to pass the oxidized oil directly to the still 12 for steam treatment, as through line 26.

It is not essential for my process to introduce the charge of untreated oil directly into the heating coil, as under certain conditions of operation I 65 found it desirable to introduce the untreated material after the coil 1 in line 2 before the still 4 through line 38, maintaining at the same time the recirculation of either air-blown asphalt by means of pump 9 and line 29, or steam-rectified asphalt 70 through pump 34 and line 36, or both, through said coil 1 and/or air-blowing still 4, by-passing, if desired, a part of that asphalt through line 48. Or I may, first, rectify the untreated material 75 with superheated steam in 12 conveying it there by means of lines 38, 24, and 11, and then oxidize

the reduced residue in a continuous operation in 4 conveying it there from 12 by means of pump 34, line 56, coil 1, and lines 39 and 2.

For the manufacture of most commercial products I operate my plant at around atmospheric pressure. However, for the making of special products it is sometimes advantageous to maintain either or both stills 4 and 12, either under pressure or vacuum; the apparatus must of course be constructed so as to be able to withstand this change 10 in conditions: special vacuum pumps may have to be added. Though usually not much vacuum or pressure is needed, I find it, under special circumstances, useful to employ considerable pressure or 15 a high vacuum.

Having fully described the details of my process and the apparatus in which the process can be successfully carried out, the invention is further defined in the appended claims.

I claim as my invention:

1. A continuous process for treating asphaltic oil to produce oxidized asphalt comprising: heating said oil to an oxidizing temperature, commingling the heated oil with an oxygen-containing gas in a confined stream, maintaining a body 25 of partly oxidized oil, discharging the said stream of the oxygen-containing gas and oil undergoing oxidation into said body, thereby causing further oxidation of the said body of oil, separating more volatile components of the oxidized oil together 30 with the residual gases of the air, withdrawing oxidized oil near the surface of said body of oil, and recirculating a portion of the withdrawn oil through the heating step.

2. A continuous process for treating an asphaltic oil to produce oxidized asphalt comprising: heating said oil to an oxidizing temperature, commingling the heated oil with an oxygen-containing gas in a confined stream, maintaining a body 40 of partly oxidized oil, discharging said stream of the oxygen-containing gas and oil undergoing oxidation into said body of oil, thereby effecting further oxidation of the body of oil, permitting the unconsumed air and more volatile components of the oxidized oil to separate from 45 the oil, withdrawing a portion of the oxidized oil, further degasifying the same, and recirculating a portion of the substantially gas-free oxidized oil through the heating step.

3. A process for treating asphaltic oil comprising maintaining a body of partly oxidized oil, withdrawing a part of said body of oil, steam rectifying at least a portion of the withdrawn oil, heating the rectified oil to an oxidizing temperature in a confined stream, mixing said stream 55 of heated oil with a stream of fresh oil, introducing an oxygen-containing gas into the combined oil stream, and discharging the resulting gas-oil stream still containing free oxygen into said body of partly oxidized oil, thereby further oxidizing 60 said body of oil.

4. A process for treating asphaltic oil comprising maintaining a body of partly oxidized oil, withdrawing a part of said body of oil, steam rectifying a portion of the withdrawn oil, commingling the rectified oil with another portion of the withdrawn oxidized oil, heating the combined oil stream to an oxidizing temperature, mixing it with a stream of fresh oil, introducing an oxygen-containing gas into the resulting oil 70 stream, and discharging the resulting gas-oil stream still containing free oxygen into said body of partly oxidized oil, thereby further oxidizing 75 said body of oil.

5. A continuous process for treating asphaltic

residual oil comprising steam-rectifying said oil in a rectifying zone, heating the rectified oil to an oxidizing temperature, commingling the heated oil with an oxygen-containing gas in a confined stream, maintaining a body of partly oxidized oil, discharging said stream into said body of oil, thereby further oxidizing said body of oil, withdrawing the oxidized oil and returning a portion thereof to the rectifying zone together with the fresh oil.

6. The process of claim 5, wherein a part of the withdrawn oxidized oil is mixed with the rectified oil and the mixture is heated to an oxidizing temperature.

7. A continuous process for treating asphaltic oil to produce oxidized asphalt, comprising: heating said oil to an oxidizing temperature, commingling the heated oil with an oxygen-containing gas in a confined stream, maintaining a body of partly oxidized oil, discharging the stream of oil and oxygen-containing gas into said body of partly oxidized oil, thereby further oxidizing the same, simultaneously separating the oxidized oil from vapors and residual gases, withdrawing and re-heating at least a portion of the resulting substantially gas-free material, and steam-rectifying said re-heated portion.

8. A continuous process for treating asphaltic oil to produce oxidized asphalt, comprising: heating said oil to an oxidizing temperature, commingling the heated oil with an oxygen-containing gas in a confined stream, maintaining a body of partly oxidized oil, discharging the stream of oil and oxygen-containing gas into said body of partly oxidized oil, thereby further oxidizing the same, simultaneously separating the oxidized oil from vapors and residual gases, withdrawing and steam-rectifying at least a portion of the resulting oxidized substantially gas-free material, commingling at least a portion of the steam-rectified liquid material with said withdrawn oxidized material, and steam-rectifying the resulting mixture.

9. A process of forming oxidized asphalt comprising: maintaining a heated bulk supply of oil in a chamber at an elevated temperature, continuously circulating substantially gas-free oil from the bulk supply to and through a heating coil and back to the bulk supply, continuously introducing an oxygen-containing gas into a con-

fined stream of the circulating oil after the oil leaves the heating coil but before it enters said chamber, commingling said stream with the oil in said chamber, continuously permitting the residual air to separate from the oil in the chamber and pass out of the system, continuously withdrawing the resulting gas-free material, re-heating it in a confined stream, and steam-rectifying said material.

10. A continuous process for treating asphaltic oil to produce oxidized asphalt comprising heating a continuous stream of fresh asphaltic oil in a heating coil in the absence of oxygen to an oxidizing temperature, commingling the heated oil while at said temperature with an oxygen-containing gas in a confined turbulent stream, maintaining a body of oxidized oil having a depth above the point of introduction of the commingled stream of oil and oxygen-containing gas effective for desired oxidation and discharging said stream of oxygen-containing gas and substantially unoxidized fresh oil into said body of oil, thereby further oxidizing said body of oil and simultaneously separating the oxidized oil while in said body from vapors and residual gases, continuously withdrawing at least a portion of the resulting substantially gas-free material oxidized to the desired extent and commingling it with the heated stream of fresh oil before it is discharged into said body of oil.

11. A continuous process for treating asphaltic oil to produce oxidized asphalt comprising heating a continuous stream of fresh asphaltic oil in a heating coil in the absence of oxygen to an oxidizing temperature, commingling the heated oil with an oxygen-containing gas in a confined turbulent stream, maintaining a body of oxidized oil having a depth above the point of introduction of the commingled stream of oil and oxygen-containing gas effective for desired oxidation and discharging said stream of oxygen-containing gas and substantially unoxidized fresh oil into said body of oil, thereby further oxidizing said body of oil and simultaneously separating the oxidized oil from vapors and residual gases, withdrawing at least a portion of the resulting substantially gas-free material oxidized to the desired extent and commingling it with the stream of fresh oil before it is subjected to heating.

ADOLF GUTZWILLER.

50